

July 13, 1965

E. KRUMBEIN ETAL

3,194,676

PRESSURE SENSITIVE TRANSFER ELEMENT

Filed Dec. 6, 1961



EDGAR KRUMBEIN  
AND  
Sig MUSCHTER  
By: NOLTE AND NOLTE  
ATTORNEYS

1

3,194,676

## PRESSURE SENSITIVE TRANSFER ELEMENT

Edgar Krumbein and Sigo Muschter, Hannover, Germany, assignors to Columbia Ribbon and Carbon Manufacturing Co., Inc., Glen Cove, N.Y.

Filed Dec. 6, 1961, Ser. No. 157,453

Claims priority, application Germany, Dec. 14, 1960, W 29,084; Mar. 16, 1961, W 29,659

10 Claims. (Cl. 117—36.1)

This invention relates to carbon and duplicating paper having a colour-spending layer based on a synthetic plastic binder material, and more particularly to the utilization of a combination of incompatible or substantially incompatible synthetic plastic binder materials for making the coating substance for such carbon and duplicating papers.

One of the most essential requirements imposed on a carbon paper the preparation of which is based on wax, as well as on synthetic materials consists in that the carbon paper should rather remain plane, and not curl when stored or during use. The carbon paper must be insensitive to possible variations of extraneous climatic conditions such as the influence of the temperature and atmospheric humidity.

Although there were not wanting proposals directed to the solution of this difficult problem, none of the efforts to neutralize the tendency toward rolling or curling by applying a wax or a synthetic resin on the back of the carbon paper have up to now led to a satisfactory result.

The present invention solves the problem by providing a novel ink-releasing coating on the front-side of the carbon paper foundation rather than by treating the back of the carbon paper foundation.

Ink-releasing layers are known which are based upon individual resinous binder materials such as vinyl chloride-vinyl acetate copolymers, or mixtures of resinous binder materials used in a ratio such they they remain compatible with each other. The compatibility of resinous materials with one another is a conventionally recognized property whereby the resins have the ability of producing optically clear solid solutions after they have been dissolved together in a mutual solvent and after the solvent has been evaporated. If the resinous materials are incompatible or are used in such a ratio that their compatibility is exceeded, then at least a portion of the resin separates from the remainder and forms a bluish or smoky appearance and loss of optical clarity in the final solid solution.

The present invention relates to the discovery that the tendency of carbon papers to curl or roll may be unexpectedly overcome by using as the binder material a mixture of synthetic resins which are at least partially incompatible with each other. The microscopic examination of the mixture invisible by an unaided eye as far as its structure is concerned shows that after the evaporation of the solvent the synthetic materials within the colour-spending layer have a superfine heterogeneous alveolar structure. The writing or printing colour matter is stored within said honeycomb-like structure and is delivered during the writing procedure in proportioned quantities so that the representation of the lettering is absolutely uniform.

According to the invention, in addition to the heterogeneity between the film-forming material (the synthetic material) and the colour matter proper existing in all known carbon papers based on synthetic materials, the present ink-releasing layers also have a very essential heterogeneity between the incompatible synthetic materials jointly used as film-forming binder materials.

In this connection it has surprisingly been discovered that a carbon and duplicating paper the colour-spending layer of which is prepared of such incompatible synthetic

2

materials and which in the finished state has a micro-porous alveolar structure does not tend toward rolling. Such a carbon paper does not require any additional means for preventing it from rolling, thereby avoiding 5 additional costs.

Also, in addition, it has been found that the colour-spending layers of the carbon paper according to the present invention distinguish themselves in that the usual disagreeable electrostatic charge is either eliminated or at 10 least reduced by far.

According to another embodiment of this invention carbon papers are provided for use in modern registering processes by including therein magnetic pigment as the coloring matter. It is known by present experience that 15 it was impossible to squeeze the magnetic pigments the average size of the particles of which is about  $0.5\mu$  out of the known microporous layers of synthetic materials. While heavy magnetizable ferric oxides are sufficiently fine as individual particles, when in solvents they tend 20 toward coagulation and thus cannot be maintained sufficiently movable in the communicating micropores of the usual layers of synthetic material. Contrary thereto, the utilization of incompatible film-forming binder-materials according to the present invention leads to the elimination 25 of the coagulation and thus to an intense lettering which has sufficient marginal sharpness and a sufficient quantity of magnetizable particles.

A few examples with respect to the preparation of the 30 film-forming material according to the present invention are set forth hereunder.

## Example 1

35 It has been found that an emulsion of equal parts of a 20% solution of a vinyl chloride-vinyl acetate copolymer and a 20% solution of a polystyrene is quite advantageous.

40 1.1 parts of reflex blue colour,  
4.5 parts of gas black,  
1.9 parts of Milori blue colour,  
0.2 part of disperser Z,  
13.1 parts of castor oil,  
45 5.6 parts of mineral oil,  
0.4 part of preservative

are pulverized in a three roller mill and intermixed within a stirring apparatus with

50 36.7 parts of a 20 percent vinyl chloride-vinyl acetate-copolymer solution (Vinoflex) and

55 36.7 parts of a polystyrene solution, whereupon the mixture is applied in a manner known per se onto the carrier material—that is, the raw paper or foil, upon thoroughly mixing the colour matter-synthetic material mixture at intervals.

60 In this connection, it is to be noted that the closer the weights of the utilized non-mixable synthetic materials to the ratio 1:1, the greater the electric neutrality of the layer. Hence it follows that in the above example, the optimum has been achieved.

## Example 2

65 By adding small parts only, of nitrocellulose or colloidion cotton, respectively, to vinyl copolymers, the writing properties of the thus obtained paper will not be impaired.

The already described effect takes place also in this case.

4.8 parts of gas black,  
2.2 parts of Milori blue colour,  
0.2 parts of disperser Z,  
18.8 parts of castor oil, and  
0.4 part of preservative

are pulverized in a three roller mill and intermixed in a turbulent stirrer with

51.6 parts of a 20 percent vinyl chloride-vinyl acetate-  
copolymer solution (Vino flex) 10

and

22.0 parts of a 15 percent solution of medium viscous  
collodion cotton in a mixture of 95% of butanone and 15  
5% of methanol,

whereupon the raw paper is coated with this mixture in  
a manner known per se.

*Example 3*

Only at most 10% of the entire content of the synthetic  
material may consist of cellulose ether, to be utilized  
with vinyl copolymers.

4.6 parts of gas black,  
2.1 parts of Milori blue colour,  
0.2 part of disperser Z,  
18.4 parts of castor oil and  
0.4 part of preservative

are pulverized and intermixed in the manner shown here-  
inabove with

60.5 parts of a 20 percent vinyl chloride-vinyl acetate-  
copolymer solution (Vino flex) 30

and

13.8 parts of an 11 percent solution of medium viscous  
ethyl cellulose in methyl ethyl ketone,

whereupon the raw paper is coated therewith in a manner  
known per se. 40

*Example 4*

The butadiene-styrene copolymers are incompatible  
with vinyl ester copolymers in any ratio. In this case,  
too, the already mentioned effect is quite pronounced.

3.6 parts of gas black,  
1.7 parts of Milori blue colour,  
0.2 part of disperser Z,  
14.2 parts of castor oil and  
0.5 part of preservative 45

are pulverized in a three roller mill and intermixed in a  
turbulent stirrer with

40.0 parts of a 20 percent vinyl chloride-vinyl acetate-  
copolymer solution (Vino flex) 50

and

40.0 parts of a 20 percent solution of a copolymer of  
butadiene and styrene in methyl ethyl ketone. 60

The examples following hereunder relate to the preparation  
of a colour component containing magnetic pigments.

*Example 5*

The colour component consists of 12 parts magnetic  
pigments S 11 (the trade name of the Farbenfabriken  
Bayer, Leverkusen, German Federal Republic). These  
parts are intermixed with 6 parts of a dehydratized  
castor oil and 4 parts of a mineral oil at three intervals  
in a three roller mill the rollers of which are spaced by  
0.03 mm.

Subsequently, the adhesive paste is stirred together with  
80 parts of a synthetic material composition according  
to the present invention (40 parts of a 20% solution of  
a vinyl chloride-vinyl acetate copolymer in methyl-ethyl-

ketone and 38 parts of a 20% polystyrene solution in  
methyl-ethyl-ketone) to a permanent dispersion, where-  
upon the mixture is applied to a carrier material in a  
manner known per se.

5 The dehydrated castor oil in connection with a mineral  
oil can be replaced by blown castor oil as a vehicle.

*Example 6*

The colour component for a carbon paper based on  
synthetic materials according to the present invention  
can also consist of a mixture of for example a PV-true  
blue B (BASF) and the magnetic pigment S 11 (the  
trade name of Farbenfabriken Bayer, Leverkusen). In  
this case, 3.5 parts of the PV-true blue (BASF) together  
with 5 parts of castor oil, 4 parts of dehydratized castor  
oil and 3 parts of mineral oils (crystal oil) are pul-  
verized at three intervals in a three-roller mill first, where-  
upon the space between the rollers is increased to 0.03  
mm. and the aforesaid mixture intimately mixed on the  
roller with 5 parts of the magnetic pigment S 11. The  
thus obtained pigment paste is stirred in the turbulent  
stirrer together with 40 parts of a solution of the syn-  
thetic material according to the invention, namely a  
20% solution of a vinyl chloride-vinyl acetate copolymer  
(Vino flex) in methyl ethyl ketone and 39.5 parts of a  
20% polystyrene solution in methyl ethyl ketone to a  
permanent dispersion.

A flexible foundation is coated with this mixture in  
a manner known per se.

A sectional view of the carbon paper according to the  
present invention in an enlarged scale is shown by way  
of example in the accompanying drawing.

The ink-releasing layer 2 consisting of a part 3 of  
synthetic binder material and of a part 4 of synthetic  
binder material is applied to a flexible foundation 1  
which may be either a paper sheet or another foil. The  
part 3 of synthetic material is a non-coherent component  
of fine particles between which there remains a free  
more or less large intermediate space. The intermediate  
spaces are filled with the part of synthetic material of the  
other component of synthetic material which forms a  
closed phase and thus produces the desired layer forma-  
tion. Both components contain capillary channels or  
pores 5 which are filled with the ink composition of the  
carbon paper. During the working procedure—that is,  
during writing, the ink composition of the carbon paper  
is squeezed out from the channels or pores 5.

What is claimed is:

1. A pressure-sensitive transfer element comprising a  
flexible foundation having thereon a microporous ink-  
releasing layer comprising as the solid binder material a  
mixture of synthetic plastic materials which are incom-  
patible in that they are incapable of forming an optically  
clear solid solution after being dissolved together in a  
mutual solvent and after the solvent has been evaporated,  
said binder material having dispersed therein a pressure-  
releasable ink comprising oil and coloring matter, the  
said mixture of incompatible synthetic plastic materials  
comprising at least about 50% by weight of a vinyl resin  
together with a sufficient incompatible amount by weight  
of a synthetic plastic material whereby the tendency of  
the ink-releasing layer to cause the transfer element to  
curl and roll is substantially completely avoided.

2. A transfer element according to claim 1 in which  
the mixture of synthetic plastic binder materials comprises  
a vinyl chloride-vinyl acetate copolymer and polystyrene  
in a ratio of about 1:1.

3. A transfer element according to claim 1 in which the  
mixture of synthetic plastic binder materials comprises  
a vinyl chloride-vinyl acetate copolymer and a butadiene  
copolymer.

4. A transfer element according to claim 1 in which  
the mixture of synthetic plastic binder materials com-  
prises a vinyl chloride-vinyl acetate copolymer and a  
cellulose ester plastic.

5. A transfer element according to claim 1 in which the synthetic plastic binder materials are present in a ratio of about 1:1.

6. A transfer element according to claim 1 in which the coloring matter comprises magnetic pigment.

7. A pressure-sensitive transfer element comprising a flexible foundation having thereon a microporous ink-releasing layer comprising as the solid binder material a mixture of substantially incompatible synthetic plastic materials having dispersed therein a pressure-releasable ink comprising oil and coloring matter, the said mixture of incompatible synthetic plastic materials comprising at least about 90% by weight of a vinyl resin together with up to about 10% by weight of a cellulose ether plastic whereby the tendency of the ink-releasing layer to cause the transfer element to curl and roll is substantially completely avoided.

8. A transfer element according to claim 7 in which the cellulose ether comprises ethyl cellulose.

9. A transfer element according to claim 7 in which

the vinyl resin comprises a vinyl chloride-vinyl acetate copolymer.

10. A transfer element according to claim 7 in which the coloring matter comprises magnetic pigment.

5

References Cited by the Examiner

UNITED STATES PATENTS

|           |      |                |       |          |
|-----------|------|----------------|-------|----------|
| 2,744,031 | 5/56 | Mumma          | ----- | 117—36.1 |
| 2,800,077 | 7/57 | Marron         | ----- | 117—36.1 |
| 2,893,890 | 7/59 | Harvey         | ----- | 117—36.1 |
| 2,943,952 | 7/60 | Clark          | ----- | 117—36.4 |
| 2,944,037 | 7/60 | Clark          | ----- | 117—36.1 |
| 2,970,926 | 2/61 | Findlay        | ----- | 117—36.1 |
| 2,984,582 | 5/61 | Newman et al.  | ----- | 117—36.4 |
| 2,989,493 | 6/61 | Clark et al.   | ----- | 117—16.1 |
| 3,029,157 | 4/62 | Sutheim et al. | ----- | 117—36.1 |
| 3,037,879 | 6/62 | Newman et al.  | ----- | 117—36.1 |

RICHARD D. NEVIUS, Primary Examiner.

20 MURRAY KATZ, WILLIAM D. MARTIN, Examiners.